

## [54] PACKAGE OF CRIMPED THERMOPLASTIC SYNTHETIC YARNS AND METHOD OF WINDING UP SAME

2,325,127 7/1943 Gladding..... 242/159  
3,450,371 6/1969 Phillips ..... 242/159

[75] Inventors: Koji Tajiri; Fumio Nagatoshi; Masateru Terano, all of Mihara, Japan

Primary Examiner—George E. Lowrance  
Assistant Examiner—Douglas B. Farrow  
Attorney, Agent, or Firm—Sherman & Shalloway

[73] Assignee: Teijin Limited, Osaka, Japan

## [57] ABSTRACT

[22] Filed: Sept. 14, 1973

A package of crimped thermoplastic synthetic yarns, and especially the polyamide type synthetic yarn, which can provide excellent knit or woven fabrics without the formation of streaks, regardless of the conditions of the winding atmosphere or the knitting or weaving atmosphere. This package has either a winding hardness of above 70° when the moisture content at its inner layered portion is less than the equilibrium moisture content at the humidity of the knitting or weaving atmosphere or a winding hardness of less than 70° when the moisture content at its inner layered portion is greater than the equilibrium moisture content at the humidity of the knitting or weaving atmosphere.

[21] Appl. No.: 397,358

## [30] Foreign Application Priority Data

Sept. 18, 1972 Japan..... 47-92847  
Nov. 1, 1972 Japan..... 47-10879

[52] U.S. Cl..... 206/392; 242/159

[51] Int. Cl..... B65d 65/16; B65d 85/04

[58] Field of Search ..... 206/392, 497; 242/159

## [56] References Cited

## 6 Claims, 3 Drawing Figures

## UNITED STATES PATENTS

1,996,791 4/1935 Blake ..... 222/159



*Fig. 2A**Fig. 2B*

**PACKAGE OF CRIMPED THERMOPLASTIC  
SYNTHETIC YARNS AND METHOD OF WINDING  
UP SAME**

This invention relates to a package of crimped thermoplastic synthetic yarn and, in particular, to a package whose hardness has been controlled in accordance with the moisture content of the yarn contained at the inner layered portion of the package to prevent the formation of streaks in the knit or woven fabrics made from the foregoing crimped yarn. The invention also relates to a method of winding up such a package.

Heretofore, in winding up crimped thermoplastic synthetic yarns onto a package, for the mere reason that when crimped yarns that have been imparted crimp by such mechanical means as the false twist crimping treatment or the stuffing crimping treatment or other means are held under high tension their crimp properties usually decline, with the consequence that the crimp properties imparted during the crimping treatment are not fully demonstrated, the usual practice was to wind up the yarn at a low tension ranging from several milligrams per denier to several tens of milligrams per denier to obtain a package of low hardness ranging between 30° and 60° (the hardness as specified by the JIS Method K6301).

However, in the case of this type of conventional package, there is the drawback that in making knit or woven fabrics by unwinding the package difficulty is experienced in obtaining knit or woven fabrics having a satisfactory hand (properties such as surface evenness and fitting property), since streaks would form in the fabric due to irregularity of the crimp development property of the crimped yarn, or the crimped yarn would not demonstrate the desired value as regards its rate of crimp development. As regards the irregularity of the crimp development property, this can be solved to a certain extent by making the atmosphere at the time of the windup of the package and that at the time of the knitting or weaving operation (especially their humidity) about the same. However, as a practical matter, while it would be possible to adjust the humidities of the yarn processing plant and the knitting or weaving plant in a rough manner, to make these humidities substantially the same would be extremely costly. Further, the adjustment of such other factors as weather or climate would be practically impossible. Again, the conventional package has such additional shortcomings as that its properties exhibit great changes depending upon the type of atmosphere it has been left to stand in, or that its unwinding property is poor. Hence, various troubles are caused by such a package during the time of its knitting or weaving.

**SUMMARY OF THE INVENTION**

A primary object of the present invention is therefore to provide a package of crimped thermoplastic synthetic yarn not having the drawbacks of the conventional package, such as hereinbefore noted, as well as a method of winding up such a package thereby making it possible to make knit or woven fabrics without streaks and of satisfactory hand.

Another object of the invention is to provide a package of crimped thermoplastic synthetic yarn in which there is no irregularity of crimp development property regardless of the differences between the humidity of the atmosphere at the time of the windup of the pack-

age and the humidity at the time of the knitting or weaving operation.

A still another object of the invention is to provide a package of crimped thermoplastic synthetic yarn which is not substantially affected by the atmosphere in which it is left to stand.

A further object is to provide a package of crimped thermoplastic synthetic yarn which demonstrates smooth unwinding properties during the time of the knitting or weaving operation.

In general, the rate of crimp development of a package of crimped thermoplastic synthetic yarns, and especially the polyamide type crimped synthetic yarn, varies depending upon the windup conditions (especially the tension at the time of the windup), as hereinbefore noted, as well as the atmospheres at the time of the windup and at the time of the knitting or weaving of the fabric (especially the humidity of the atmospheres).

As a result of our detailed researches as to what effects the tension at the time of the windup and the humidities at the time of the windup and at the time of the knitting or weaving operation would have on the rate of crimp development of the crimped yarn, as well as our recognition that the irregularity of the rate of crimp development is based on the difference in the moisture content of the crimped yarn between the inner layered portion and the outer layered portion of the package, we found that if the tension at the time of the windup is adjusted to a prescribed value the irregularity of the rate of crimp development could be eliminated and at the same time the desired rate of crimp development could be obtained even though there is a difference between the humidity at the time of the windup and either the humidity at which the yarn was left to stand or the humidity at the time of the knitting or weaving operation.

Thus, there is provided according to this invention a package of crimped thermoplastic synthetic yarn which is characterized in that the package either has a winding hardness of 70° to 95° when the moisture content of the yarn at the inner layered portion of the package is less than the equilibrium moisture content at the relative humidity of the atmosphere to be used at the time of the knitting or weaving operation or has a winding hardness of less than 70° when the moisture content of the yarn at the inner layered portion of the package is greater than the equilibrium moisture content at the relative humidity of the atmosphere to be used at the time of knitting or weaving operation.

There is further provided according to this invention a method of winding up a package of crimped thermoplastic synthetic yarn, the method comprising either winding up the yarn at a winding tension of at least 0.15 gram per denier while adjusting the relative humidity of the winding atmosphere at below the relative humidity of the atmosphere to be used at the time of the knitting or weaving operation or winding up the yarn at a winding tension less than 0.15 gram per denier while adjusting the relative humidity of the winding atmosphere at above the relative humidity of the atmosphere to be used at the time of the knitting or weaving operation.

**BRIEF DESCRIPTION OF THE DRAWINGS**

The invention will be more fully described hereinafter with reference being had to the accompanying drawings, in which:

FIG. 1 is a graph showing how changes take place in the rate of crimp development depending upon the winding tension and the winding humidity; and

FIGS. 2-A and 2-B are schematic views illustrating the forces that act on the yarn when a false twist formed crimped yarn wound up on a pirln package is being unwound from the package.

#### DETAILED DESCRIPTION OF THE PREFERRED EMBODIMENT

The moisture content of a thermoplastic synthetic yarn, and especially the polyamide type synthetic yarn, usually changes in accordance with the humidity of its surrounding atmosphere. In the case of a wound package, the outer layered portions (i.e., the peripheral portion, and in the case of the pirln package, the tapered portion, or in the case of the cheese package, the two end portions) achieve an equilibrium moisture content corresponding to the relative humidity of the atmosphere surrounding the package while, on the other hand, there is practically no change in the moisture content of the inner layered portion of the package, a moisture content corresponding to the relative humidity at the time of the windup being maintained over a prolonged period of time. Hence, a difference occurs in the moisture contents of the inner layered portion and the outer layered portion of the package in correspondence with the difference between the relative humidity of the atmosphere surrounding the package, generally the atmosphere at the time of the knitting or weaving operation, and the relative humidity at the time of the windup. An example will be given for explaining this difference in moisture contents. When a 20 denier 6 filament yarn of nylon is submitted to a false twist treatment in which the number of false twists is 6000 T/m and heat-setting temperature is 180°C., following which the yarn is wound up on a pirln, this yarn has a moisture content of about 3.0 percent. Now, when this package is left standing in an atmosphere of 20°C. and relative humidity of 65 percent, the moisture content of the inner layered portion of this package shows practically no change, but the outer layered portion (i.e., the peripheral and tapered portions) changes to an equilibrium moisture content relative to the atmosphere in which it is left standing of 4.2 percent.

The moisture content is obtained in the following manner. After sampling about 5 grams of the yarn, its weight  $W_1$  is determined, following which the yarn is air dried for 3 hours at 105°C. The dried yarn is then cooled in a desiccator, after which its weight  $W_2$  is determined. The moisture content is then calculated as follows:

$$\text{Moisture content} = W_1 - W_2/W_2 \times 100 \text{ (percent)}$$

In the case of the polyamide type crimped synthetic yarn, the rate of column development at the time the package is being unwound, as hereinafter fully described, becomes smaller at that portion where the moisture content is high as compared with that portion where the moisture content is low. Hence, in the case such as hereinabove described, the rate of crimp development of the crimped yarn of the tapered portion of the pirln package becomes less than that of the crimped yarn of the inner layered portion of the package, with the consequence that the apparent bulkiness of this portion in the knit or woven fabric becomes smaller than the other portions of the fabric to result in formation of streaks.

By the expression "inner layered portion" of the package, as used herein, is meant the crimped yarn layer portion located at a depth of at least 2 centimeters from the surface of the package, while the expression "outer layered portion" of the package denotes that portion located within 5 millimeters of the surface of the package.

While the rate of crimp development of the crimped yarn varies depending upon its moisture content as hereinbefore noted, it also is greatly influenced by the winding tension that is applied during the windup as explained hereinafter by reference to FIG. 1.

FIG. 1, wherein the winding tension is represented as abscissa and the rate of crimp development is represented as ordinate, graphically shows the changes in the rate of crimp development when the moisture content and the winding tension (and hence the hardness of the package) are varied, the moisture content of the crimped yarn being varied in this case by varying the humidity surrounding the crimped yarn (either the humidity of the winding atmosphere or the humidity at which the package is left to stand). The rate of crimp development shown in FIG. 1 was obtained in the following manner. That is, the wound package was left to stand for about two weeks to stabilize its moisture content and tension. The crimped yarn was then sampled from the package onto a reel of about 40-cm size under a tension of 0.15 gram per denier at a temperature and humidity corresponding to the atmosphere that would be encountered during the knitting or weaving operation, the size of the sample crimped yarn being made about 1900 denier. The sample was then applied a load of 2 mg per denier and the length of the hank  $l$  was measured 2 minutes later. A further load of 0.1 gram per denier was applied, and the length of the hank  $l_0$  was measured 2 minutes later. The rate of crimp development was then calculated as follows:

Crimp development rate =  $l_0 - l/l_0 \times 100$  (percent)  
The rate of crimp development obtained in this manner corresponds satisfactorily with the amount of crimp that develops during the knitting or weaving operation. When the dispersion of this value exceeds 10 percent, it was found that streaks would form in the knit or woven product.

When a detailed examination of FIG. 1 is made, the following facts are revealed. First of all, it was considered that the rate of crimp development would decline when the yarn was wound up under high tension, and hence it was the practice to carry out the winding at a low tension of several mg per denier to several tens of mg per denier to obtain a package of low hardness, i.e., one having a hardness of 30° to 60° (a value determined with a spring type rubber hardness meter as specified by the JIS Method K6301). However, it can be seen that there was rather a decline in the rate of crimp development with such a low tension and it is seen that contrary to the experience there is surprisingly an increase in the rate of crimp development when the hardness of the package was made more than 70° by winding up the package at a high tension of above 0.15 gram per denier. To be sure, as can be seen from FIG. 1, a large rate of crimp development is also demonstrated when the winding tension is a very low value of close to zero, but as a practical matter in the case of a low tension such as this the winding density becomes exceedingly small and the package would collapse during

its handling and transportation. Hence, a low tension such as this is of no practical use.

The reason that, as noted above, the rate of crimp development becomes small when the windup is carried out at low tension, such as practiced in the past, but increase when the windup is performed at a considerably high tension is conceivably due to the fact that the fibers shrink at low tension and the shrinkage acts to decrease the curvature of the crimps, whereas at high tension, the shrinkage is not permitted and with stretching of such a degree, there is a complete elastic recovery. Accordingly, when the windup is carried out at low tension, crimps are not developed during weaving or knitting to worsen the stretchability and surface evenness, whereas in the high tension windup, crimps are well developed during weaving or knitting to improve the stretchability and surface evenness of the resulting woven or knitted fabric.

Next, referring to FIG. 1, an examination of the relationship between the winding humidity of the crimped yarn (and hence its moisture content) and the rate of crimp development will be made. In the first place, it can be seen that the lower the winding humidity, the higher the rate of crimp development that is obtained. This is conceivably due to the following reason. When the crimped yarn is one whose moisture content is lower than the equilibrium moisture content relative to the knitting or weaving atmosphere, the yarn on becoming free as a result of having been unwound from the package absorbs moisture at the same time. Now, the plasticizing effect of this moisture has a promotional effect on the release of the tension, with the consequence that the development of crimps is enhanced. On the other hand, in the case of a crimped yarn having a higher moisture content than the equilibrium moisture content relative to the knitting or weaving atmosphere, the yarn on becoming free as a result of having been unwound from the package discharges moisture, with the consequence that the plasticizing effect due to the moisture is lost and hence the development of crimps becomes less.

On further examination of FIG. 1, the following fact will become apparent. That is, in the case where the winding humidity is greater than the knitting or weaving humidity (i.e., where the moisture content of the crimped yarn is greater than the equilibrium humidity relative to the knitting or weaving atmosphere), if the windup is carried out at a tension less than 0.15 gram per denier, there is an area where fluctuations in the rate of crimp development ascribable to the difference of the moisture content of the crimped yarn are exceedingly small.

Further, when the winding humidity is less than the knitting or weaving humidity (i.e., where the moisture content of the crimped yarn is less than the equilibrium moisture content relative to the knitting or weaving atmosphere), quite a contrary phenomenon occurs, and it is seen that when the windup is carried out at a tension of above 0.15 gram per denier, and preferably above 0.25 grams per denier, fluctuations in the rate of crimp development ascribable to the difference of the moisture content of the crimped yarn are slight.

These tendencies, as seen in FIG. 1, were substantially the same even when the relative humidity of the knitting or weaving room was varied.

The fact that the difference in the rate of crimp development ascribable to the difference of moisture con-

tent is slight means that the allowable range of fluctuations in relative humidity at the time of processing becomes wide, and moreover, even though a difference in the moisture contents between the inner layered portion and the outer layered portion of a package occur, i.e., even though there is a difference in the winding humidity and the knitting or weaving humidity, since there is only a slight difference in the rate of crimp development, there is no formation of irregularities in the knit or woven product.

When the foregoing observations in connection with FIG. 1 are coordinated, an appreciation of the following facts will be had.

1. When the moisture content of the inner layered portion of the package (this corresponds to the winding humidity) is adjusted at less than the equilibrium moisture content relative to the knitting or weaving atmosphere (this corresponds to the knitting or weaving humidity) and the crimped yarn is wound up at a winding tension of above 0.15 gram per denier, and preferably above 0.25 gram per denier, to obtain a package having a hardness of at least 70°, and preferably at least 80°, not only can the rate of crimp development be enhanced, but also its difference ascribable to the difference between the winding humidity and the knitting or weaving humidity can be reduced. However, if the winding tension employed is too great, plastic deformation will be set up in the crimped yarn as a result of its elastic limit being exceeded. Hence, the upper limit of the winding tension should preferably be set at 1.0 g per denier, preferably 0.7 gram per denier.

2. When the moisture content of the inner layered portion of the package is adjusted at above the equilibrium moisture content relative to the knitting or weaving atmosphere and the crimped yarn is wound up at a winding tension less than 0.15 gram per denier to obtain a package having a hardness of less than 70°, the rate of crimp development is small but the fluctuations in the rate of crimp development ascribable to the difference between the winding humidity and the knitting or weaving humidity can be made very small.

Hence, it will be seen that, provided the package is either one in which the moisture content of the inner layered portion is less than the equilibrium moisture content at the relative humidity of the knitting or weaving atmosphere and which has a winding hardness of above 70°, and preferably 80° to 95°, or one in which the moisture content of the inner layered portion is above the equilibrium moisture content at the relative humidity of the knitting or weaving atmosphere and which has a winding hardness of less than 70°, it is possible to make knit or woven products having no streaks.

Again, when a product having a high rate of crimp development is desired from the standpoint of its hand, etc., it is possible to form a package that can make the desired knit or woven product by adjusting the humidity of the winding atmosphere at less than the humidity of the knitting or weaving atmosphere to be used and winding up the yarn at a winding tension of above 0.15 gram per denier to 1.0 gram per denier, and preferably from 0.25 gram per denier to 0.7 gram per denier.

As hereinbefore noted, the thermoplastic synthetic fibers, and especially the polyamide type synthetic fibers, are susceptible to the influence of the humidity of the surrounding atmosphere, and while the fibers at the inner layered portion of the package maintains the moisture content that is determined by the humidity of

the atmosphere at the time of winding of the package, the moisture content of the fibers at the outer layered portion of the package changes to that determined by the humidity of the atmosphere at which the package is left to stand. Hence, the outer layered portion of the package is adversely affected depending upon the conditions at which it is left to stand from the time of its winding to the time it is used in the knitting or weaving operation, with the consequence that there arises the possibility of causing the formation of streaks in the knit or woven product.

It is thus preferred that the package, after its formation, be hermetically packed with a moisture-impermeable material under an atmosphere identical to that under which the package was formed, thus ensuring that the outer layered portion of the package is not affected by the atmosphere at which the package is left to stand.

As the procedure to be used for accomplishing this hermetical packing, that of fuse-sealing the package using as the moisture-impermeable material a thermoplastic polymeric material such as polyethylene or polypropylene is preferred. However, good results are had even by such a procedure as placing the package in a bag prepared from a moisture-impermeable material and closing the opening of the bag with a rubber band or the like.

Now, of the crimped thermoplastic synthetic yarns, the false twist crimped yarn which has been imparted crimps by false twisting, as a finished yarn of greatest versatility at the present time, is being used in various areas such as for outer garments, underwear, socks and women's hosiery, panty hosiery, etc., but this false twist crimped yarn possesses torques as well as crimps as an inevitable result of the principles by which the crimping process operates. At times, troubles are experienced during the unwinding of the package on account of this torque. This will be explained by reference to FIG. 2-A. FIG. 2-A illustrates the case of a pirln package that has been wound up in the Z direction by imparting a true twist to the false twist crimped yarn having an S twist. As shown in FIG. 2-A, the yarn receives at the unwinding point 1 a force A upwardly of the bobbin as a result of the unwinding operation. On the other hand, the yarn possesses a torque due to the falst twist, as noted above. Since the package has been wound up in the Z direction by imparting a true twist to the crimped yarn having a falst twist in the S direction, this torque has a force B which rolls in an upward direction over the surface of the pirln package. Hence, the force A resulting from the unwinding and the sorce B ascribable to the torque act in substantially the same direction to cause not only an excessive unwinding of the yarn but also a slipping off of the yarn from the tapered portion in the form of a loop, after which this loop becomes entangled as a result of the torque. This entanglement then either gets introduced into the knit or woven fabric before it has been unravelled to greatly impair the quality of the fabric or becomes caught on the needles or other parts of the knitting or weaving machine to cause yarn breakage. This tendency is especially marked when the unwinding point 1 has arrived in the vicinity of the upper tapered portion of the package.

FIG. 2-B illustrates the case of a pirln package consisting of false twist crimped yarn of S twist which has been wound up by rotating the bobbin in the S direction. When this package is being unwound, the yarn re-

ceives at its unwinding point a force C in the upward direction of the bobbin. On the other hand, the torque ascribable to the false twist and having a rolling force in the S direction comes to have in the case of this package of FIG. 2-B a force D rolling over the surface of the package towards the bottom of the bobbin. Since the forces C and D act against each other, these force offset each other, with the consequence that troubles such as occur in the case of the package shown in FIG. 2-A do not arise.

Thus, it will be appreciated from the foregoing discussion that in the case where a false twist crimped yarn having torque is to be wound up on a package it is preferred that the winding is carried out such that the torque acting on the yarn as a result of the false twist becomes at the unwinding point a force rolling in a direction opposite to that of the force acting on the yarn as a result of the unwinding of the yarn.

While the case of a pirln package has been illustrated and explained, the foregoing explanation also apply equally to the case of such other packages as the cheese and cone packages. However, since, in the case of the pirln package, there is a recessed portion at the bottom of the bobbin for engaging, say, the spindle of a ring twisting apparatus, or there is a protector covering the exposed metallic part, or the yarn end for which the winding step was started remains, difficulty is experienced in unwinding the yarn towards the bottom of the bobbin axis, and thus the unwinding is usually carried out towards the upper part of the bobbin axis. Hence, in the case of the pirln package, for achieving a smooth unwinding of the yarn as hereinabove described, it is necessary to carry out the winding of the yarn by rotating the bobbin in the same direction as that used in false twisting the yarn in the crimping treatment.

#### EXAMPLE 1

A 20 denier/6 filament drawn yarn of nylon 6 was imparted crimps by the conventional crimping process, after which the yarn was wound up by varying the winding tensions as well as the relative humidities of the winding chamber to prepare several packages having inner layered portions of varying moisture contents. These packages were left standing for over a day in knitting rooms of varying relative humidities to prepare several classes of packages whose inner layered portions and outer layered portions had varying moisture contents. These packages were then knit into stockings under the conditions at which they were left to stand, and the surface evenness and, the fitting property were examined. While the surface evenness of the knit product can be clearly discerned by visual inspection, since difficulty is experienced in expressing their evaluation with numerical values, the symbols O, Δ, X will be used in evaluating this property. The symbol O denotes that the surface evenness is excellent, while the symbol X denotes that the surface evenness is unsatisfactory. On the other hand, the symbol Δ denotes that the surface evenness is intermediate between that of the symbol O and that of the symbol X. The fitting property is evaluated by the length of the stocking immediately after its knitting, as measured from below the welt of the thigh portion to the toe. The shorter this length is, the more satisfactory is the fitting property. The moisture content was determined in the following manner. A given amount of the sample is taken and weighed ( $W_1$ ), following which the sample is dried for 3 hours at 105°C.

and thereafter cooled for 40 minutes in a desiccator containing silica gel. The sample is then weighed ( $W_2$ ) again, and the moisture content is calculated as follows:

$$\text{Moisture content} = W_1 - W_2/W_2 \times 100 \text{ (percent)}$$

On the other hand, the package hardness was determined with a spring type hardness tester Model A in accordance with the JIS Method K6301. The results obtained are shown in Table 1.

Table 1

| Sample No. | Winding chamber humidity (RH %) | Winding tension (g/de) | Knitting room humidity (RH %) | Hardness (°C.) | Moisture content (%)  |                       |                  | Length of stocking (mm) | Presence of streaks |
|------------|---------------------------------|------------------------|-------------------------------|----------------|-----------------------|-----------------------|------------------|-------------------------|---------------------|
|            |                                 |                        |                               |                | Inner layered portion | Outer layered portion | Surface evenness |                         |                     |
| 1          | 49                              | 0.04                   | 64                            | 60             | 3.0                   | 4.2                   | X                | 610                     | Yes                 |
| 2          | 49                              | 0.15                   | 64                            | 75             | 3.0                   | 4.2                   | O - Δ            | 560                     | No                  |
| 3          | 49                              | 0.35                   | 64                            | 85             | 3.0                   | 4.2                   | O                | 510                     | No                  |
| 4          | 49                              | 0.5                    | 64                            | 95             | 3.0                   | 4.2                   | O                | 490                     | No                  |
| 5          | 68                              | 0.03                   | 49                            | 60             | 4.5                   | 3.0                   | X                | 710                     | No                  |
| 6          | 50                              | 0.04                   | 49                            | 60             | 3.0                   | 3.0                   | X                | 660                     | No                  |
| 7          | 69                              | 0.3                    | 49                            | 85             | 4.5                   | 3.0                   | X                | 630                     | Yes                 |
| 8          | 62                              | 0.4                    | 44                            | 90             | 4.0                   | 2.6                   | X                | 640                     | Yes                 |
| 9          | 56                              | 0.4                    | 56                            | 90             | 3.5                   | 3.5                   | Δ - O            | 580                     | No                  |
| 10         | 49 - 60                         | 0.4                    | 64                            | 90             | 3.0-3.8               | 4.2                   | O                | 520                     | No                  |
| 11         | 68 - 79                         | 0.4                    | 64                            | 90             | 4.5-5.3               | 4.2                   | Δ                | 600                     | Yes                 |
| 12         | 49 - 60                         | 0.04                   | 64                            | 60             | 3.0-3.8               | 4.2                   | X                | 640                     | Yes                 |
| 13         | 68 - 79                         | 0.03                   | 64                            | 60             | 4.5-5.3               | 4.2                   | X                | 700                     | No                  |

In the first place, it is seen from Table 1 that in the case of the stockings knit from a package having a hardness of above 70° and in which the moisture content of the inner layered portion (the equilibrium moisture content relative to the humidity of the winding chamber) was less than the moisture content of the outer layered portion (the equilibrium moisture content relative to the humidity of the knitting or weaving room), i.e., packages in accordance with the present invention (Samples 2, 3, 4, 9 and 10), the hand (surface evenness and fitting property) was satisfactory and, in addition, no streaks were present. Next, in the case of the stockings knit from a package having a hardness of less than 70° and in which the moisture content of the inner layered portion was less than that of the outer layered portion (Samples 1 and 12), the formation of streaks was noted. On the other hand, in the case of the stocking knit from the package having a hardness of above 70° and in which the moisture content of the inner layered portion was greater than the outer layered portion (Samples 7, 8 and 11), it can be seen that the product was slightly inferior with respect to both its hand and presence of streaks.

Packages (Samples No. 5, 6 and 13) having an inner layer moisture content greater than the outer layer moisture content and a hardness of not more than 70° have difficulty of developing streaks, but there is a de-

fect that the surface unevenness and fitting property are reduced.

Furthermore, as is seen by comparing Sample No. 10 with Samples Nos. 11 and 12, when the hardness is above 70°, and the inner layer moisture content is less than the moisture content of the outer layer, streaks are scarcely formed even if the moisture content of the

inner layer, namely the windup humidity, fluctuates to some degree.

## EXAMPLE 2

The false twisting treatment of a 64 denier/6 filament undrawn yarn of nylon 6 was carried out under the conditions of false twists numbering 6200 T/m and a heater temperature of 185°C., using a drawing and frictional type false twister. In carrying out this false twisting treatment, the winding tension at the time of the windup was carried by varying the weight of the traveler and the rpm of the spindle. At the same time, the hardness of the package and its moisture content were varied by varying the relative humidity of the winding portion. The so obtained samples having varying moisture contents and winding tensions were left to stand for at least one day in knitting rooms of given relative humidities (50 and 60 percent) and were thus conditioned so that there would be a difference in the moisture contents of the inner layered and outer layered portions of the pirl. The so prepared packages were then fed to a 4-feeder seamless stocking knitting machine in an atmosphere identical to that at which they were left to stand. The stocking obtained from these packages were then examined for streaks, with the results shown in Table 2. The moisture content and hardness were determined as in Example 1.

Table 2

| Sample No. | Winding chamber humidity (RH %) | Winding tension (g/de) | Knitting room humidity (RH %) | Hardness (°C.) | Moisture content (%)  |                       |                  | Presence of streaks |
|------------|---------------------------------|------------------------|-------------------------------|----------------|-----------------------|-----------------------|------------------|---------------------|
|            |                                 |                        |                               |                | Inner layered portion | Outer layered portion | Surface evenness |                     |
| 1          | 65                              | 0.07                   | 64                            | 62             | 4.2                   | 4.2                   | X                | No                  |
| 2          | 70                              | 0.07                   | 64                            | 63             | 4.6                   | 4.2                   | X                | No                  |
| 3          | 80                              | 0.07                   | 64                            | 65             | 5.3                   | 4.2                   | X                | No                  |
| 4          | 50                              | 0.07                   | 64                            | 63             | 3.1                   | 4.2                   | X                | Yes                 |
| 5          | 40                              | 0.07                   | 64                            | 61             | 2.3                   | 4.2                   | X                | Yes                 |
| 6          | 65 - 75                         | 0.3                    | 64                            | 90             | 4.3 - 5.0             | 4.2                   | X                | Yes                 |
| 7          | 66 - 75                         | 0.06                   | 64                            | 60             | 4.3 - 5.0             | 4.2                   | X                | No                  |
| 8          | 65                              | 0.1                    | 54                            | 66             | 4.2                   | 3.4                   | X                | No                  |
| 9          | 55 - 70                         | 0.1                    | 54                            | 67             | 3.5 - 4.6             | 3.4                   | X                | No                  |
| 10         | 40                              | 0.1                    | 54                            | 66             | 2.3                   | 3.4                   | X                | Yes                 |
| 11         | 50 - 40                         | 0.1                    | 54                            | 68             | 3.1 - 2.3             | 3.4                   | X                | Yes                 |
| 12         | 55 - 70                         | 0.4                    | 54                            | 92             | 3.5 - 4.6             | 3.4                   | X                | Yes                 |

It is seen from Table 2 that stockings knit from packages having a hardness of less than 70° and in which the moisture content of the inner layered portion was greater than that of the outer layered portion, i.e., packages in accordance with the present invention, (Samples 1, 2, 3, 7, 8 and 9) had no streaks. On the other hand, in the case of the stockings knit from packages having a hardness of above 70° and in which the moisture content of the inner layered portion was greater than that of the outer layered portion (Samples 6 and 12) as well as the stockings knit from packages having a hardness of less than 70° and in which the moisture content of the inner layered portion was less than that of the outer layered portion (Samples 4, 5, 10 and 11), it is seen that there were formations of streaks.

We claim:

1. A package of a crimped yarn of thermoplastic synthetic fibers, said package either being one having a winding hardness of above 70° when the moisture content of the yarn at the inner layered portion of the package is less than the equilibrium moisture content at the relative humidity of the atmosphere to be used at the time of the knitting or weaving operation or being one having a winding hardness of less than 70° when the moisture content of the yarn at the inner lay-

20  
25

ered portion of the package is greater than the equilibrium moisture content at the relative humidity of the atmosphere to be used at the time of the knitting or weaving operation.

5. A package according to claim 1 wherein said crimped yarn of thermoplastic synthetic fibers is of a polyamide type synthetic fiber.

3. A package according to claim 2, said package having a winding hardness of above 70°, the moisture content of the inner layered portion of said package being adjusted such that it is less than the equilibrium moisture content at the relative humidity of the atmosphere to be used at the time of the knitting or weaving operation.

15. 4. A package according to claim 3 in which the winding hardness of the package is from 80° to 95°.

5. A package according to claim 2 wherein said package is hermetically wrapped with an impervious material.

20. 6. A package according to claim 5 wherein said impervious material is a thermoplastic high molecular substance, said package being fuse-sealed by said material.

\* \* \* \* \*

30

35

40

45

50

55

60

65